

# United States Patent [19]

Hashimoto et al.

[11] Patent Number: 4,481,271

[45] Date of Patent: Nov. 6, 1984

[54] LAYERED ELECTROPHOTOGRAPHIC  
PHOTOCONDUCTOR CONTAINING A  
HYDRAZONE

[75] Inventors: Mitsuru Hashimoto; Kiyoshi Sakai; Toshio Fukagai, all of Numazu, Japan; Tatsuya Katoh, deceased, late of Tokyo, Japan, by Tazuko Katoh, heir; by Mankichi Katoh, legal representative, Yokohama, Japan

[73] Assignee: Ricoh Company, Ltd., Tokyo, Japan

[21] Appl. No.: 330,548

[22] Filed: Dec. 14, 1981

[30] Foreign Application Priority Data

Dec. 15, 1980 [JP] Japan ..... 55-176913  
Dec. 15, 1980 [JP] Japan ..... 55-176914  
Dec. 15, 1980 [JP] Japan ..... 55-176915  
Dec. 15, 1980 [JP] Japan ..... 55-176916  
Dec. 15, 1980 [JP] Japan ..... 55-176917  
Dec. 15, 1980 [JP] Japan ..... 55-176918  
Dec. 15, 1980 [JP] Japan ..... 55-176919  
Dec. 15, 1980 [JP] Japan ..... 55-176920  
Dec. 19, 1980 [JP] Japan ..... 55-178748  
Dec. 19, 1980 [JP] Japan ..... 55-178749  
Dec. 19, 1980 [JP] Japan ..... 55-178750  
Dec. 19, 1980 [JP] Japan ..... 55-178751  
Dec. 19, 1980 [JP] Japan ..... 55-178752  
Dec. 19, 1980 [JP] Japan ..... 55-178760  
Dec. 19, 1980 [JP] Japan ..... 55-178761

[51] Int. Cl. 3 ..... G03G 5/06

[52] U.S. Cl. ..... 430/57; 430/58;  
430/59; 430/72

[58] Field of Search ..... 430/57, 58, 59, 72

[56] References Cited

U.S. PATENT DOCUMENTS

4,150,987 4/1979 Anderson et al. ..... 430/58  
4,327,168 4/1982 Hashimoto ..... 430/57  
4,390,608 6/1983 Hashimoto et al. ..... 430/57

Primary Examiner—John D. Welsh

Attorney, Agent, or Firm—Flynn, Thiel, Boutell & Tanis

[57] ABSTRACT

A layered electrophotographic photoconductor whose

charge generation layer comprises a bisazo pigment selected from the group consisting of the bisazo pigments represented by the following general formula (I) and whose charge transport layer contains a charge transport material selected from the group consisting of the hydrazone compounds represented by the following general formula (2):



wherein A represents  $-C_6H_4-Cl(o)$ ,  $-C_6H_4-Cl(m)$ ,  $-C_6H_4-Br(o)$ ,  $-C_6H_4-Br(m)$ ,  $-C_6H_4-F(o)$ ,  $-C_6H_4-F(m)$ ,  $-C_6H_4-F(p)$ , or  $-C_6H_4-I(m)$ ,



wherein R<sup>1</sup> represents a substituted or non-substituted naphthyl group, a substituted or non-substituted anthryl group, a substituted or non-substituted styryl group, or



wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other; R<sup>2</sup> represents an alkyl group, a benzyl group; and R<sup>3</sup> represents a phenyl group or a methoxyphenyl group.

16 Claims, 1 Drawing Figure

U.S. Patent

Nov. 6, 1984

4,481,271



# LAYERED ELECTROPHOTOGRAPHIC PHOTOCOMPONENT CONTAINING A HYDRAZONE

## BACKGROUND OF THE INVENTION

The present invention relates to a layered electrophotographic photoconductor comprising an electroconductive support material and a photoconductive double layer which consists of a charge generation layer and a charge transport layer. In particular, it is concerned with a layered electrophotographic photoconductor whose charge generation layer comprises a bisazo pigment selected from the group consisting of the bisazo pigments represented by the following general formula (1) and whose charge transport layer contains a charge transport material selected from the group consisting of the hydrazone compounds represented by the following general formula (2):



wherein A represents  $-\text{C}_6\text{H}_4-\text{Cl}(\text{o})$ ,  $-\text{C}_6\text{H}_4-\text{Cl}(\text{m})$ ,  $-\text{C}_6\text{H}_4-\text{Br}(\text{o})$ ,  $-\text{C}_6\text{H}_4-\text{Br}(\text{m})$ ,  $-\text{C}_6\text{H}_4-\text{F}(\text{o})$ ,  $-\text{C}_6\text{H}_4-\text{F}(\text{m})$ ,  $-\text{C}_6\text{H}_4-\text{F}(\text{p})$ , or  $-\text{C}_6\text{H}_4-\text{I}(\text{m})$ ;



wherein R<sup>1</sup> represents a substituted or non-substituted naphthyl group, a substituted or non-substituted anthryl group, a substituted or non-substituted styryl group, or



wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other; R<sup>2</sup> represents an alkyl group, a benzyl group; and R<sup>3</sup> represents a phenyl group or a methoxyphenyl group.

Conventionally, a variety of inorganic and organic 5  
electrophotographic photoconductors are known. As  
inorganic electrophotographic photoconductors, there  
are known, for instance, a selenium photoconductor, a  
selenium-alloy photoconductor, and a zinc oxide photo-  
conductor which is prepared by sensitizing zinc oxide 6  
with a sensitizer pigment and dispersing the same in a  
binder resin. Furthermore, as a representative example  
of organic electrophotographic photoconductors, an  
electrophotographic photoconductor comprising a  
complex of 2,4,7-trinitro-9-fluorenone and poly-N- 6  
vinylcarbazole is known.

However, while these electrophotographic photoconductors have many advantages over other conven-

tional electrophotographic photoconductors, at the same time they have several shortcomings from the viewpoint of practical use.

For instance, a selenium photoconductor which is widely used at present has the shortcomings that its production is difficult and, accordingly, its production cost is high, and due to its poor flexibility, it is difficult to work into the form of a belt. Furthermore, it is so vulnerable to heat and mechanical shock that it must be handled with the utmost care.

In contrast to this, the zinc oxide photoconductor is inexpensive since it can be produced more easily than the selenium photoconductor. Specifically, it can be produced by simply coating inexpensive zinc oxide particles on a support material. However, it is poor in photosensitivity, surface smoothness, hardness, tensile strength and wear resistance. Therefore, it is not suitable for a photoconductor for use in plain paper copiers in which the photoconductor is used in quick repetition.

20 The photoconductor employing the aforementioned complex of 2,4,7-trinitro-9-fluorenone and poly-N-vinylcarbazole is also poor in photosensitivity and is therefore not suitable for practical use, particularly for 25 a high speed copying machine.

Recently, extensive studies have been done on the electrophotographic photoconductors of the above-mentioned types, in order to eliminate the above-described shortcomings of the conventional photoconductors. In particular, attention has focused on layered organic electrophotographic photoconductors, each comprising an electroconductive support layer, a charge generation layer comprising an organic pigment formed on the electroconductive support layer, and a charge transport layer comprising a charge transport material formed on the charge generation layer, which are for use in plain paper copiers, since such layered organic electrophotconductors have high photosensitivity and stable charging properties. As a matter of fact, some type of layered electrophotographic photoconductors are being successfully used in practice. Examples of the layered electrophotographic photoconductors are as follows:

45 (1) U.S. Pat. No. 3,871,882 discloses a layered electro-photographic photoconductor whose charge generation layer comprises a perylene derivative and whose charge transport layer comprises an oxadiazole derivative.

50 (2) Japanese Laid-open Patent Applications No. 52-55643 and No. 52-72231 disclose a layered electro-photographic photoconductor whose charge generation layer comprises Chlorodiane Blue which is dispersed in an organic amine and coated on an electroconductive support material and whose charge transfer 55 layer comprises a pyrazoline derivative.

(3) Japanese Laid-open Patent Application No. 53-95033 discloses a layered electrophotographic photoconductor whose charge generation layer comprises a carbazole type bisazo pigment dispersed, for instance, in tetrahydrofuran and coated on an electroconductive support material, and whose charge transport layer comprises 2,5-bis(4-diethylaminophenyl)-1,3,4-oxadiazole or TNF.

65 (4) Japanese Laid-open Patent Application No. 54-12742 discloses a layered electrophotographic photoconductor of the same type as that disclosed in Japanese Laid-open Patent Application No. 53-95033, in

which the carbazole type bisazo pigment is replaced by an oxadizole type bisazo pigment.

(5) Japanese Laid-open Patent Application No. 54-22834 also discloses a layered electrophotographic photoconductor of the same type as that disclosed in Japanese Laid-open Patent Application No. 53-95033, in which the carbazole type bisazo pigment is replaced by a fluorenone type bisazo pigment.

As mentioned previously, these layered electrophotographic photoconductors have many advantages over other electrophotographic photoconductors, but at the same time, they have a variety of shortcomings.

Specifically, the electrophotographic photoconductor (1) employing a perylene derivative and an oxadizole derivative presents no problem for use in an ordinary electrophotographic copying machine, but its photosensitivity is insufficient for use in a high speed electrophotographic copying machine. Furthermore, since the perylene derivative, which is a charge generation material and has the function of controlling the spectral sensitivity of the photoconductor, does not necessarily have spectral absorbance in the entire visible region, this photoconductor cannot be employed for use in color copiers.

The electrophotographic photoconductor (2) employing Chlorodiane Blue and a pyrazoline derivative exhibits comparatively good photosensitivity. However, when preparing that photoconductor, an organic amine, for example, ethylene diamine, which is difficult to handle, is necessary as a coating solvent for forming the charge generation layer.

The electrophotographic photoconductors (3) through (5), for which the inventors of the present invention applied for patents, have an advantage over other conventional electrophotographic photoconductors in that the charge generation layers can be prepared easily by coating the dispersions of fine particles of the pigments in an organic solvent (with addition of a binder resin thereto when necessary) on an electroconductive support material. However, the photosensitivities of the photoconductors (3) through (5) are so low that that they cannot be used as photoconductors for high speed electrophotographic copiers.

#### SUMMARY OF THE INVENTION

It is therefore an object of the present invention to provide a layered electrophotographic photoconductor comprising an electroconductive support material and a photoconductive double layer which consists of a charge generation layer and a charge transport layer, with high photosensitivity and uniform spectral absorbance in the visible region, and which gives rise to no difficulty in production of the electrophotographic photoconductor.

According to the present invention, the charge generation layer comprises a bisazo pigment selected from the group consisting of the bisazo pigments represented by the following general formula (1), and the charge transport layer comprises a charge transport material selected from the group consisting of the hydrazone compounds represented by the following general formula (2):



wherein A represents  $-C_6H_4-Cl(o)$ ,  $-C_6H_4-Cl(m)$ ,  $-C_6H_4-Br(o)$ ,  $-C_6H_4-Br(m)$ ,  $-C_6H_4-F(o)$ ,  $-C_6H_4-F(m)$ ,  $-C_6H_4-F(p)$ , or  $-C_6H_4-I(m)$ ;

15

20



wherein R<sup>1</sup> represents a substituted or non-substituted naphthyl group, a substituted or non-substituted anthryl group, a substituted or non-substituted styryl group, or

25

30

35

40

45

50



wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other; R<sup>2</sup> represents an alkyl group, a benzyl group; and R<sup>3</sup> represents a phenyl group or a methoxyphenyl group.

According to the present invention, by the layered construction of the charge generation layer and the charge transport layer, which respectively comprises the above-mentioned charge generating material and the charge transporting material, and by the particular combination of the charge generating material and the charge transporting material, there is provided an electrophotographic photoconductor capable of providing high surface potential in the dark and dissipating the surface potential speedily upon exposure to light and without any substantial change in electrophotographic properties during repeated electrophotographic copying, which copying process includes charging, exposure, development and elimination of latent electrostatic images by charge quenching.

#### BRIEF DESCRIPTION OF THE DRAWING

In the drawing, the single FIGURE shows an enlarged cross section of a layered electrophotographic photoconductor according to the present invention.

#### DETAILED DESCRIPTION OF THE PREFERRED EMBODIMENTS

60

65

Referring to the single FIGURE, there is shown an enlarged cross section of an embodiment of a layered electrophotographic photoconductor according to the present invention. As shown in this FIGURE, a charge generation layer 22 comprising a charge generating material is formed on an electroconductive support material 11, and a charge transport layer 33 comprising a charge transporting material is formed on the charge generation layer 22. The charge generation layer 22 and

charge transport layer 33 constitute a photoconductive layer 44 as shown in the FIGURE.

In the thus formed layered electrophotographic photoconductor, a latent electrostatic image is formed by the following mechanism:

The surface of the layered electrophotographic photoconductor is electrically charged uniformly in the dark, so that electric charges are formed in the surface of the photoconductor. The thus electrically charged photoconductor is then exposed to an optical image. When this exposure is done, the rays of light of the optical image pass through the transparent charge transport layer 33 and enter the charge generation layer 22 where the rays of light are then absorbed by the charge generating material present in the charge generation layer 22. Upon absorption of the rays of light, the charge generating material generates charge carriers, which are then injected into the charge transport layer 33. The injected charge carriers are transported towards the surface of the photoconductor through the charge transport layer 33 in accordance with the electric field applied thereto by the first mentioned electric charging, so that electric charges present in the surface of the photoconductor are neutralized, whereby a latent electrostatic image is formed on the surface of the photoconductor.

Referring to the FIGURE, the electroconductive support material 11 for use in the present invention can be made of a plate, drum or foil of metals, such as aluminum, nickel or chromium; a plastic film with a thin layer of aluminum, tin oxide, indium, chromium or palladium; or a sheet of paper or plastic film with an electrically conductive material coated thereon, or impregnated with an electrically conductive material.

The charge generation layer 22 is formed on the electroconductive support material 11 by grinding a bisazo pigment, which works as the charge generating material and which is represented by the formula (1), into fine particles, for instance by a ball mill, and dispersing the fine particles of the bisazo pigment in a solvent, if necessary with the addition of a binder resin to the dispersion, and coating that dispersion on the electroconductive support material 11.



wherein A represents  $-\text{C}_6\text{H}_4-\text{Cl}(\text{o})$ ,  $-\text{C}_6\text{H}_4-\text{Cl}(\text{m})$ ,  $-\text{C}_6\text{H}_4-\text{Br}(\text{o})$ ,  $-\text{C}_6\text{H}_4-\text{Br}(\text{m})$ ,  $-\text{C}_6\text{H}_4-\text{F}(\text{o})$ ,  $-\text{C}_6\text{H}_4-\text{F}(\text{m})$ ,  $-\text{C}_6\text{H}_4-\text{F}(\text{p})$ , or  $-\text{C}_6\text{H}_4-\text{I}(\text{m})$ .

When necessary, the surface of the charge generation layer 22 is made smooth or the thickness of the charge generation layer 22 is adjusted by buffing.

The thickness of the charge generation layer 22 is in the range of  $0.01 \mu\text{m}$  to  $5 \mu\text{m}$ , preferably in the range of  $0.05 \mu\text{m}$  to  $2 \mu\text{m}$ , and the content of the bisazo compound in the charge generation layer 22 is in the range of 10 weight percent to 100 weight percent, preferably in the range of 30 weight percent to 95 weight percent.

When the thickness of the charge generation layer 22 is less than  $0.01 \mu\text{m}$ , the photosensitivity of the electrophotographic photoconductor is insufficient for practical use, while when the thickness of the charge generation layer 22 is more than  $5 \mu\text{m}$ , the charge retention

property of this photoconductor becomes poor. Furthermore, when the content of the bisazo pigment in the charge generation layer 22 is less than 10 weight percent, the photoconductor does not exhibit sufficiently high photosensitivity for practical use.

The charge transport layer 33 is formed on the charge generation layer 22 by coating thereon a tetrahydrofuran solution of the hydrazone compound represented by the formula (2) and a binder resin.



15 wherein  $\text{R}^1$  represents a substituted or non-substituted naphthyl group, a substituted or non-substituted anthryl group, a substituted or non-substituted styryl group, or



20 25 wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other;  $\text{R}^2$  represents an alkyl group, a benzyl group; and  $\text{R}^3$  represents a phenyl group or a methoxyphenyl group.

The content of the hydrazone compound in the charge transport layer 33 is in the range of 10 weight percent to 80 weight percent, preferably in the range of 25 weight percent to 75 weight percent.

The thickness of the charge transport layer 33 is in the range of  $2 \mu\text{m}$  to  $100 \mu\text{m}$ , preferably in the range of  $5 \mu\text{m}$  to  $40 \mu\text{m}$ .

40 45 When the content of the hydrazone compound in the charge transport layer 33 is less than 10 weight percent, the photosensitivity of this photoconductor is poor, while when the content of the hydrazone compound is more than 80 percent, the charge transport layer 33 becomes brittle or the hydrazone compound contained in the charge transport layer 33 separates out in the form of crystals, making the charge transport layer 33 opaque and having adverse effects on the electrophotographic properties of the photoconductor.

50 55 When the thickness of the charge transport layer 33 is less than  $5 \mu\text{m}$ , the surface potential cannot be retained properly, while when the thickness of the charge transport layer 33 is more than  $40 \mu\text{m}$ , the residual potential of the photoconductor tends to become too high for practical use.

As the binder resin for use in the charge generation layer 22, a polyester resin, a butyral resin, an ethyl cellulose resin, an epoxy resin, an acrylic resin, a polyvinylidene resin, polystyrene, polybutadiene chloride resin and copolymers of those resins can be used individually or in combinations thereof.

60 65 As the binder resin for use in the charge transport layer 33, a polycarbonate resin, a polyester resin, polystyrene, polybutadiene, a polyurethane resin, an epoxy resin, an acrylic resin, a silicone resin and copolymers of those resins can be used individually or in combinations thereof.

Furthermore, in order to improve the flexibility and mechanical strength of the charge transport layer 33, a variety of additives, such as halogenated paraffin, dialkyl phthalate and silicone oil can be added to the charge transport layer 33.

In the present invention, when necessary, a barrier layer can be disposed between the electroconductive support material 11 and the charge generation layer 22, an intermediate layer between the charge generation

layer 22 and the charge transport layer 33, or an overcoat layer on top of the charge transport layer 33.

In the present invention, the following bisazo compounds are particularly useful, which are represented by the previously described general formula (1), in combination with one of the following hydrazone compounds represented by the previously described general formula (2) in the above-described layered photoconductor.

Bisazo Compounds



-continued  
Bisazo Compounds



Hydrazone Compounds



-continued  
Hydrazone Compounds



-continued  
Hydrazone Compounds



(2-4) 5

10



(2-5) 15

20



(2-6) 25

30



(2-7) 35

35



(2-8) 40

40



(2-9) 45

45



(2-10) 50

55



(2-11) 60

60



(2-12) 65

65

-continued  
Hydrazone Compounds

(2-13)

(2-14)

(2-15)

(2-16)

(2-17)

-continued



-continued

Hydrazone Compounds

-continued

Hydrazone Compounds

(2-30) 5



10

(2-31) 15



20

(2-32)



35

(2-33)



45

(2-34)



55

(2-35)



65

(2-36)

(2-37)

(2-38)

(2-39)

(2-40)

(2-41)

-continued  
Hydrazone Compounds



(2-42)

10  
15

(2-43)

20  
25

(2-44)

30  
35

(2-45)

40  
45

(2-46)

50  
55

(2-47)

60  
65

-continued  
Hydrazone Compounds



(2-48)



(2-49)



(2-50)



(2-51)



(2-52)



(2-53)

-continued  
Hydrazone Compounds



Embodiments of a layered electrophotographic photoco conductor according to the present invention will now be explained.

## EXAMPLE 1

## (Layered Photoconductor No. 1-1)

One part by weight of a bisazo compound represented by the formula (1-1), 19 parts by weight of tetrahydrofuran, and 6 parts by weight of a tetrahydrofuran solution of a polyvinyl butyral resin (Trade name: XYHL made by Union Carbide Plastic Company) (5 weight percent) were ground in a ball mill.

To the thus ground mixture were added, with slow stirring, 104 parts by weight of tetrahydrofuran. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 13.1  $\mu\text{m}$  was formed on the charge generation layer, whereby a layered electrophotographic photoconductor No. 1-1 was prepared.

## EXAMPLE 2

## (Layered Photoconductor No. 1-2)

Example 1 was repeated except that hydrazone compound (2-14) was replaced with hydrazone compound (2-4), so that a layered electrophotographic photoconductor No. 1-2 with a charge generation layer with a thickness of 0.8  $\mu\text{m}$  and a charge transport layer with a thickness of 17.9  $\mu\text{m}$  was prepared.

## EXAMPLE 3

## (Layered Photoconductor No. 1-3)

Example 1 was repeated except that the polyvinyl butyral resin was replaced with a polyester resin (Trade Name: Vylon 200 made by Toyobo Co., Ltd.), so that a layered electrophotographic photoconductor No. 1-3 with a charge generation layer with a thickness of 0.8  $\mu\text{m}$  and a charge transport layer with a thickness of 16.5  $\mu\text{m}$  was prepared.

## EXAMPLE 4

## (Layered Photoconductor No. 1-4)

Example 1 was repeated except that hydrazone compound (2-14) was replaced with hydrazone compound (2-3), so that a layered electrophotographic photoconductor No. 1-4 with a charge generation layer with a thickness of 0.8  $\mu\text{m}$  and a charge transport layer with a thickness of 18.0  $\mu\text{m}$  was prepared.

## EXAMPLE 5

## (Layered Photoconductor No. 2-1)

One part by weight of a bisazo compound represented by the formula (1-2), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 15.2  $\mu\text{m}$  was formed on the charge generation layer, whereby a layered electrophotographic photoconductor No. 2-1 was prepared.

## EXAMPLE 6

## (Layered Photoconductor No. 2-2)

Example 5 was repeated except that hydrazone compound (2-14) was replaced with hydrazone compound (2-4), so that a layered electrophotographic photoconductor No. 2-2 with a charge generation layer with a thickness of 0.8  $\mu\text{m}$  and a charge transport layer with a thickness of 18.2  $\mu\text{m}$  was prepared.

## EXAMPLE 7

## (Layered Photoconductor No. 2-3)

Example 5 was repeated except that the polyvinyl butyral resin was replaced with a polyester resin (Trade Name: Vylon 200 made by Toyobo Co., Ltd.), so that a layered electrophotographic photoconductor No. 2-3 with a charge generation layer with a thickness of 0.8

$\mu\text{m}$  and a charge transport layer with a thickness of 17.4  $\mu\text{m}$  was prepared.

## EXAMPLE 8

(Layered Photoconductor No. 3-1)

One part by weight of a bisazo compound represented by the formula (1-3), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 12.7  $\mu\text{m}$  was formed on the charge generation layer, whereby a layered electrophotographic photoconductor No. 3-1 was prepared.

## EXAMPLE 9

(Layered Photoconductor No. 3-2)

Example 8 was repeated except that hydrazone compound (2-14) was replaced with hydrazone compound (2-4), so that a layered electrophotographic photoconductor No. 3-2 with a charge generation layer with a thickness of 1.0  $\mu\text{m}$  and a charge transport layer with a thickness of 18.3  $\mu\text{m}$  was prepared.

## EXAMPLE 10

(Layered Photoconductor No. 4-1)

One part by weight of a bisazo compound represented by the formula (1-4), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 part by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then

at 100° C. for 5 minutes, so that a charge transport layer with a thickness of 17.1  $\mu\text{m}$  was formed on the charge generation layer, whereby a layered electrophotographic photoconductor No. 4-1 was prepared.

## EXAMPLE 11

(Layered Photoconductor No. 4-2)

Example 10 was repeated except that hydrazone compound (2-14) was replaced with hydrazone compound (2-4), so that a layered electrophotographic photoconductor No. 4-2 with a charge generation layer with a thickness of 0.9  $\mu\text{m}$  and a charge transport layer with a thickness of 21.2  $\mu\text{m}$  was prepared.

## EXAMPLE 12

(Layered Photoconductor No. 4-3)

Example 10 was repeated except that the polyvinyl butyral resin was replaced with a polyester resin (Trade Name: Vylon 200 made by Toyobo Co., Ltd.), so that a layered electrophotographic photoconductor No. 4-3 with a charge generation layer with a thickness of 0.9  $\mu\text{m}$  and a charge transport layer with a thickness of 20.9  $\mu\text{m}$  was prepared.

## EXAMPLE 13

(Layered Photoconductor No. 5-1)

One part by weight of a bisazo compound represented by the formula (1-5), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 15.7  $\mu\text{m}$  was formed on the charge generation layer, whereby a layered electrophotographic photoconductor No. 5-1 was prepared.

## EXAMPLE 14

(Layered Photoconductor No. 5-2)

Example 13 was repeated except that hydrazone compound (2-4) was replaced with hydrazone compound (2-4), so that a layered electrophotographic photoconductor No. 5-2 with a charge generation layer with a thickness of 0.8  $\mu\text{m}$  and a charge transport layer with a thickness of 18.1  $\mu\text{m}$  was prepared.

## EXAMPLE 15

(Layered Photoconductor No. 5-3)

Example 13 was repeated except that the polyvinyl butyral resin was replaced with a polyester resin (Trade Name: Vylon 200 made by Toyobo Co., Ltd.), so that a layered electrophotographic photoconductor No. 5-3 with a charge generation layer with a thickness of 0.8  $\mu\text{m}$  and a charge transport layer with a thickness of 17.2  $\mu\text{m}$  was prepared.

## EXAMPLE 16

(Layered Photoconductor No. 6-1)

One part by weight of a bisazo compound represented by the formula (1-6), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 1.0  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 13.5  $\mu\text{m}$  was formed on the charge generation layer, whereby a layered electrophotographic photoconductor No. 6-1 was prepared.

## EXAMPLE 17

(Layered Photoconductor No. 6-2)

Example 16 was repeated except that hydrazone compound (2-14) was replaced with hydrazone compound (2-4), so that a layered electrophotographic photoconductor No. 6-2 with a charge generation layer with a thickness of 1.0  $\mu\text{m}$  and a charge transport layer with a thickness of 18.0  $\mu\text{m}$  was prepared.

## EXAMPLE 18

(Layered Photoconductor No. 7-1)

One part by weight of a bisazo compound represented by the formula (1-7), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 17.4  $\mu\text{m}$  was formed on the charge generation layer, whereby a layered electrophotographic photoconductor No. 7-1 was prepared.

## EXAMPLE 19

(Layered Photoconductor No. 7-2)

Example 18 was repeated except that hydrazone compound (2-14) was replaced with hydrazone compound (2-4), so that a layered electrophotographic photoconductor No. 7-2 with a charge generation layer with a thickness of 0.9  $\mu\text{m}$  and a charge transport layer with a thickness of 17.2  $\mu\text{m}$  was prepared.

## EXAMPLE 20

(Layered Photoconductor No. 7-3)

Example 18 was repeated except that the polyvinyl butyral resin was replaced with a polyester resin (Trade Name: Vylon 200 made by Toyobo Co., Ltd.), so that a layered electrophotographic photoconductor No. 7-3 with a charge generation layer with a thickness of 0.9  $\mu\text{m}$  and a charge transport layer with a thickness of 17.7  $\mu\text{m}$  was prepared.

## EXAMPLE 21

(Layered Photoconductor No. 8-1)

One part by weight of a bisazo compound represented by the formula (1-8), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-14), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 14.2  $\mu\text{m}$  was formed on the charge generation layer, whereby a layered electrophotographic photoconductor No. 8-1 was prepared.

## EXAMPLE 22

(Layered Photoconductor No. 8-2)

Example 21 was repeated except that hydrazone compound (2-14) was replaced with hydrazone compound (2-4), so that a layered electrophotographic photoconductor No. 8-3 with a charge generation layer with a thickness of 0.8  $\mu\text{m}$  and a charge transport layer with a thickness of 18.1  $\mu\text{m}$  was prepared.

## EXAMPLE 23

(Layered Photoconductor No. 8-3)

Example 21 was repeated except that the polyvinyl butyral resin was replaced with a polyester resin (Trade Name: Vylon 200 made by Toyobo Co., Ltd.), so that a layered electrophotographic photoconductor No. 8-3 with a charge generation layer with a thickness of 0.8  $\mu\text{m}$  and a charge transport layer with a thickness of 17.1  $\mu\text{m}$  was prepared.

## EXAMPLE 24

(Layered Photoconductor No. 9-1)

One part by weight of a bisazo compound represented by the formula (1-1), 19 parts by weight of tetrahydrofuran, and 6 parts by weight of a tetrahydrofuran solution of a polyvinyl butyral resin (Trade name: XYHL made by Union Carbide Plastic Company) (5 weight percent) were ground in a ball mill.

To the thus ground mixture were added, with slow stirring, 104 parts by weight of tetrahydrofuran. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 16.3  $\mu\text{m}$  was formed on the charge generation layer, whereby a layered electrophotographic photoconductor No. 9-1 was prepared.

## EXAMPLE 25

(Layered Photoconductor No. 9-2)

Example 24 was repeated except that hydrazone compound (2-26) was replaced with hydrazone compound (2-20), so that a layered electrophotographic photoconductor No. 9-2 with a charge generation layer with a thickness of 0.9  $\mu\text{m}$  and a charge transport layer with a thickness of 17.4  $\mu\text{m}$  was prepared.

## EXAMPLE 26

(Layered Photoconductor No. 9-3)

Example 24 was repeated except that hydrazone compound (2-26) was replaced with hydrazone compound (2-36), so that a layered electrophotographic photoconductor No. 9-3 with a charge generation layer

with a thickness of 0.9  $\mu\text{m}$  and a charge transport layer with a thickness of 18.2  $\mu\text{m}$  was prepared.

## EXAMPLE 27

(Layered Photoconductor No. 9-4)

Example 24 was repeated except that hydrazone compound (2-26) was replaced with hydrazone compound (2-23), so that a layered electrophotographic photoconductor No. 9-4 with a charge generation layer with a thickness of 0.9  $\mu\text{m}$  and a charge transport layer with a thickness of 16.3  $\mu\text{m}$  was prepared.

## EXAMPLE 28

(Layered Photoconductor No. 9-5)

Example 24 was repeated except that hydrazone compound (2-26) was replaced with hydrazone compound (2-30), so that a layered electrophotographic photoconductor No. 9-5 with a charge generation layer with a thickness of 0.9  $\mu\text{m}$  and a charge transport layer with a thickness of 15.7  $\mu\text{m}$  was prepared.

## EXAMPLE 29

(Layered Photoconductor No. 9-6)

Example 24 was repeated except that hydrazone compound (2-26) was replaced with hydrazone compound (2-24), so that a layered electrophotographic photoconductor No. 9-5 with a charge generation layer with a thickness of 0.9  $\mu\text{m}$  and a charge transport layer with a thickness of 20.3  $\mu\text{m}$  was prepared.

## EXAMPLE 30

(Layered Photoconductor No. 9-7)

Example 24 was repeated except that the polyvinyl butyral resin was replaced with a polyester resin (Trade Name: Vylon 200 made by Toyobo Co., Ltd.), so that a layered electrophotographic photoconductor No. 9-7 with a charge generation layer with a thickness of 0.9  $\mu\text{m}$  and a charge transport layer with a thickness of 18.1  $\mu\text{m}$  was prepared.

## EXAMPLE 31

(Layered Photoconductor No. 10-1)

One part by weight of a bisazo compound represented by the formula (1-2), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer

with a thickness of 17.2  $\mu\text{m}$  was formed on the charge generation layer, whereby a layered electrophotographic photoconductor No. 10-1 was prepared.

#### EXAMPLE 32

##### (Layered Photoconductor No. 10-2)

Example 31 was repeated except that hydrazone compound (2-26) was replaced with hydrazone compound (2-20), so that a layered electrophotographic photoconductor No. 10-2 with a charge generation layer with a thickness of 0.8  $\mu\text{m}$  and a charge transport layer with a thickness of 17.5  $\mu\text{m}$  was prepared.

#### EXAMPLE 33

##### (Layered Photoconductor No. 10-3)

Example 31 was repeated except that hydrazone compound (2-26) was replaced with hydrazone compound (2-36), so that a layered electrophotographic photoconductor No. 10-3 with a charge generation layer with a thickness of 0.8  $\mu\text{m}$  and a charge transport layer with a thickness of 18.0  $\mu\text{m}$  was prepared.

#### EXAMPLE 34

##### (Layered Photoconductor No. 10-4)

Example 31 was repeated except that hydrazone compound (2-26) was replaced with hydrazone compound (2-23), so that a layered electrophotographic photoconductor No. 10-4 with a charge generation layer with a thickness of 0.8  $\mu\text{m}$  and a charge transport layer with a thickness of 17.1  $\mu\text{m}$  was prepared.

#### EXAMPLE 35

##### (Layered Photoconductor No. 10-5)

Example 31 was repeated except that hydrazone compound (2-26) was replaced with hydrazone compound (2-30), so that a layered electrophotographic photoconductor No. 10-5 with a charge generation layer with a thickness of 0.8  $\mu\text{m}$  and a charge transport layer with a thickness of 16.3  $\mu\text{m}$  was prepared.

#### EXAMPLE 36

##### (Layered Photoconductor No. 10-6)

Example 31 was repeated except that hydrazone compound (2-26) was replaced with hydrazone compound (2-24), so that a layered electrophotographic photoconductor No. 10-6 with a charge generation layer with a thickness of 0.8  $\mu\text{m}$  and a charge transport layer with a thickness of 19.8  $\mu\text{m}$  was prepared.

#### EXAMPLE 37

##### (Layered Photoconductor No. 10-7)

Example 32 was repeated except that the polyvinyl butyral resin was replaced with a polyester resin (Trade Name: Vylon 200 made by Toyobo Co., Ltd.), so that a layered electrophotographic photoconductor No. 10-7 with a charge generation layer with a thickness of 0.8  $\mu\text{m}$  and a charge transport layer with a thickness of 18.0  $\mu\text{m}$  was prepared.

#### EXAMPLE 38

##### (Layered Photoconductor No. 11-1)

One part by weight of a bisazo compound represented by the formula (1-3), 19 parts by weight of tetrahydrofuran, and 6 parts by weight of a tetrahydrofuran solution of a polyvinyl butyral resin (Trade Name:

XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 1.1  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 17.3  $\mu\text{m}$  was formed on the charge generation layer, whereby a layered electrophotographic photoconductor No. 11-1 was prepared.

#### EXAMPLE 39

##### (Layered Photoconductor No. 11-2)

Example 38 was repeated except that hydrazone compound (2-26) was replaced with hydrazone compound (2-20), so that a layered electrophotographic photoconductor No. 11-2 with a charge generation layer with a thickness of 0.9  $\mu\text{m}$  and a charge transport layer with a thickness of 18.6  $\mu\text{m}$  was prepared.

#### EXAMPLE 40

##### (Layered Photoconductor No. 11-3)

Example 38 was repeated except that hydrazone compound (2-26) was replaced with hydrazone compound (2-36), so that a layered electrophotographic photoconductor No. 11-3 with a charge generation layer with a thickness of 0.9  $\mu\text{m}$  and a charge transport layer with a thickness of 18.0  $\mu\text{m}$  was prepared.

#### EXAMPLE 41

##### (Layered Photoconductor No. 11-4)

Example 38 was repeated except that hydrazone compound (2-26) was replaced with hydrazone compound (2-23), so that a layered electrophotographic photoconductor No. 11-4 with a charge generation layer with a thickness of 0.9  $\mu\text{m}$  and a charge transport layer with a thickness of 17.6  $\mu\text{m}$  was prepared.

#### EXAMPLE 42

##### (Layered Photoconductor No. 11-5)

Example 38 was repeated except that hydrazone compound (2-26) was replaced with hydrazone compound (2-30), so that a layered electrophotographic photoconductor No. 11-5 with a charge generation layer with a thickness of 1.0  $\mu\text{m}$  and a charge transport layer with a thickness of 16.0  $\mu\text{m}$  was prepared.

#### EXAMPLE 43

##### (Layered Photoconductor No. 11-6)

Example 38 was repeated except that hydrazone compound (2-26) was replaced with hydrazone compound (2-24), so that a layered electrophotographic photoconductor No. 11-6 with a charge generation

layer with a thickness of 1.0  $\mu\text{m}$  and a charge transport layer with a thickness of 19.3  $\mu\text{m}$  was prepared.

## EXAMPLE 44

## (Layered Photoconductor No. 12-1)

One part by weight of a bisazo compound represented by the formula (1-4), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 part by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 20.4  $\mu\text{m}$  was formed on the charge generation layer, whereby a layered electrophotographic photoconductor No. 12-1 was prepared.

## EXAMPLE 45

## (Layered Photoconductor No. 12-2)

Example 44 was repeated except that hydrazone compound (2-26) was replaced with hydrazone compound (2-20), so that a layered electrophotographic photoconductor No. 12-2 with a charge generation layer with a thickness of 0.9  $\mu\text{m}$  and a charge transport layer with a thickness of 21.0  $\mu\text{m}$  was prepared.

## EXAMPLE 46

## (Layered Photoconductor No. 12-3)

Example 44 was repeated except that hydrazone compound (2-26) was replaced with hydrazone compound (2-36), so that a layered electrophotographic photoconductor No. 12-3 with a charge generation layer with a thickness of 0.9  $\mu\text{m}$  and a charge transport layer with a thickness of 22.0  $\mu\text{m}$  was prepared.

## EXAMPLE 47

## (Layered Photoconductor No. 12-4)

Example 44 was repeated except that hydrazone compound (2-26) was replaced with hydrazone compound (2-23), so that a layered electrophotographic photoconductor No. 12-4 with a charge generation layer with a thickness of 0.9  $\mu\text{m}$  and a charge transport layer with a thickness of 19.5  $\mu\text{m}$  was prepared.

## EXAMPLE 48

## (Layered Photoconductor No. 12-5)

Example 44 was repeated except that hydrazone compound (2-26) was replaced with hydrazone compound (2-30), so that a layered electrophotographic photoconductor No. 12-5 with a charge generation

layer with a thickness of 0.9  $\mu\text{m}$  and a charge transport layer with a thickness of 22.5  $\mu\text{m}$  was prepared.

## EXAMPLE 49

## (Layered Photoconductor No. 12-6)

Example 44 was repeated except that hydrazone compound (2-26) was replaced with hydrazone compound (2-24), so that a layered electrophotographic photoconductor No. 12-6 with a charge generation layer with a thickness of 0.9  $\mu\text{m}$  and a charge transport layer with a thickness of 19.4  $\mu\text{m}$  was prepared.

## EXAMPLE 50

## (Layered Photoconductor No. 12-7)

Example 45 was repeated except that the polyvinyl butyral resin was replaced with a polyester resin (Trade Name: Vylon 200 made by Toyobo Co., Ltd.), so that a layered electrophotographic photoconductor No. 12-7 with a charge generation layer with a thickness of 0.9  $\mu\text{m}$  and a charge transport layer with a thickness of 19.6  $\mu\text{m}$  was prepared.

## EXAMPLE 51

## (Layered Photoconductor No. 13-1)

One part by weight of a bisazo compound represented by the formula (1-5), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.8  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 17.1  $\mu\text{m}$  was formed on the charge generation layer, whereby a layered electrophotographic photoconductor No. 13-1 was prepared.

## EXAMPLE 52

## (Layered Photoconductor No. 13-2)

Example 51 was repeated except that hydrazone compound (2-26) was replaced with hydrazone compound (2-20), so that a layered electrophotographic photoconductor No. 13-2 with a charge generation layer with a thickness of 0.8  $\mu\text{m}$  and a charge transport layer with a thickness of 18.2  $\mu\text{m}$  was prepared.

## EXAMPLE 53

## (Layered Photoconductor No. 13-3)

Example 51 was repeated except that hydrazone compound (2-26) was replaced with hydrazone compound (2-36), so that a layered electrophotographic

photoconductor No. 13-3 with a charge generation layer with a thickness of 0.8  $\mu\text{m}$  and a charge transport layer with a thickness of 18.5  $\mu\text{m}$  was prepared.

## EXAMPLE 54

## (Layered Photoconductor No. 13-4)

Example 51 was repeated except that hydrazone compound (2-26) was replaced with hydrazone compound (2-23), so that a layered electrophotographic photoconductor No. 13-4 with a charge generation layer with a thickness of 0.8  $\mu\text{m}$  and a charge transport layer with a thickness of 17.7  $\mu\text{m}$  was prepared.

## EXAMPLE 55

## (Layered Photoconductor No. 13-5)

Example 51 was repeated except that hydrazone compound (2-26) was replaced with hydrazone compound (2-30), so that a layered electrophotographic photoconductor No. 13-5 with a charge generation layer with a thickness of 0.8  $\mu\text{m}$  and a charge transport layer with a thickness of 16.3  $\mu\text{m}$  was prepared.

## EXAMPLE 56

## (Layered Photoconductor No. 13-6)

Example 51 was repeated except that hydrazone compound (2-26) was replaced with hydrazone compound (2-24), so that a layered electrophotographic photoconductor No. 13-6 with a charge generation layer with a thickness of 0.8  $\mu\text{m}$  and a charge transport layer with a thickness of 19.2  $\mu\text{m}$  was prepared.

## EXAMPLE 57

## (Layered Photoconductor No. 13-7)

Example 52 was repeated except that the polyvinyl butyral resin was replaced with a polyester resin (Trade Name: Vylon 200 made by Toyobo Co., Ltd.), so that a layered electrophotographic photoconductor No. 13-7 with a charge generation layer with a thickness of 0.8  $\mu\text{m}$  and a charge transport layer with a thickness of 18.7  $\mu\text{m}$  was prepared.

## EXAMPLE 58

## (Layered Photoconductor No. 14-1)

One part by weight of a bisazo compound represented by the formula (1-6), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 1.0  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then

at 100° C. for 5 minutes, so that a charge transport layer with a thickness of 17.0  $\mu\text{m}$  was formed on the charge generation layer, whereby a layered electrophotographic photoconductor No. 14-1 was prepared.

## EXAMPLE 59

## (Layered Photoconductor No. 14-2)

Example 58 was repeated except that hydrazone compound (2-26) was replaced with hydrazone compound (2-20), so that a layered electrophotographic photoconductor No. 14-2 with a charge generation layer with a thickness of 0.9  $\mu\text{m}$  and a charge transport layer with a thickness of 17.8  $\mu\text{m}$  was prepared.

## EXAMPLE 60

## (Layered Photoconductor No. 14-3)

Example 58 was repeated except that hydrazone compound (2-26) was replaced with hydrazone compound (2-36), so that a layered electrophotographic photoconductor No. 14-3 with a charge generation layer with a thickness of 1.0  $\mu\text{m}$  and a charge transport layer with a thickness of 17.6  $\mu\text{m}$  was prepared.

## EXAMPLE 61

## (Layered Photoconductor No. 14-4)

Example 58 was repeated except that hydrazone compound (2-26) was replaced with hydrazone compound (2-23), so that a layered electrophotographic photoconductor No. 14-4 with a charge generation layer with a thickness of 0.9  $\mu\text{m}$  and a charge transport layer with a thickness of 17.0  $\mu\text{m}$  was prepared.

## EXAMPLE 62

## (Layered Photoconductor No. 14-5)

Example 58 was repeated except that hydrazone compound (2-26) was replaced with hydrazone compound (2-30), so that a layered electrophotographic photoconductor No. 14-5 with a charge generation layer with a thickness of 0.9  $\mu\text{m}$  and a charge transport layer with a thickness of 16.3  $\mu\text{m}$  was prepared.

## EXAMPLE 63

## (Layered Photoconductor No. 14-6)

Example 58 was repeated except that hydrazone compound (2-26) was replaced with hydrazone compound (2-24), so that a layered electrophotographic photoconductor No. 14-6 with a charge generation layer with a thickness of 0.9  $\mu\text{m}$  and a charge transport layer with a thickness of 19.1  $\mu\text{m}$  was prepared.

## EXAMPLE 64

## (Layered Photoconductor No. 15-1)

One part by weight of a bisazo compound represented by the formula (1-7), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture was added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge

generation layer with a thickness of 0.9  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 16.8  $\mu\text{m}$  was formed on the charge generation layer, whereby a layered electrophotographic photoconductor No. 15-1 was prepared.

#### EXAMPLE 65

##### (Layered Photoconductor No. 15-2)

Example 64 was repeated except that hydrazone compound (2-26) was replaced with hydrazone compound (2-20), so that a layered electrophotographic photoconductor No. 15-2 with a charge generation layer with a thickness of 0.9  $\mu\text{m}$  and a charge transport layer with a thickness of 16.9  $\mu\text{m}$  was prepared.

#### EXAMPLE 66

##### (Layered Photoconductor No. 15-3)

Example 64 was repeated except that hydrazone compound (2-26) was replaced with hydrazone compound (2-36), so that a layered electrophotographic photoconductor No. 15-3 with a charge generation layer with a thickness of 0.9  $\mu\text{m}$  and a charge transport layer with a thickness of 19.2  $\mu\text{m}$  was prepared.

#### EXAMPLE 67

##### (Layered Photoconductor No. 15-4)

Example 64 was repeated except that hydrazone compound (2-26) was replaced with hydrazone compound (2-23), so that a layered electrophotographic photoconductor No. 15-4 with a charge generation layer with a thickness of 0.9  $\mu\text{m}$  and a charge transport layer with a thickness of 15.5  $\mu\text{m}$  was prepared.

#### EXAMPLE 68

##### (Layered Photoconductor No. 15-5)

Example 64 was repeated except that hydrazone compound (2-26) was replaced with hydrazone compound (2-30), so that a layered electrophotographic photoconductor No. 15-5 with a charge generation layer with a thickness of 0.9  $\mu\text{m}$  and a charge transport layer with a thickness of 17.8  $\mu\text{m}$  was prepared.

#### EXAMPLE 69

##### (Layered Photoconductor No. 15-6)

Example 64 was repeated except that hydrazone compound (2-26) was replaced with hydrazone compound (2-24), so that a layered electrophotographic photoconductor No. 15-6 with a charge generation layer with a thickness of 0.9  $\mu\text{m}$  and a charge transport layer with a thickness of 19.1  $\mu\text{m}$  was prepared.

#### EXAMPLE 70

##### (Layered Photoconductor No. 15-7)

Example 65 was repeated except that the polyvinyl butyral resin was replaced with a polyester resin (Trade Name: Vylon 200 made by Toyobo Co., Ltd.), so that a

layered electrophotographic photoconductor No. 15-7 with a charge generation layer with a thickness of 0.9  $\mu\text{m}$  and a charge transport layer with a thickness of 17.7  $\mu\text{m}$  was prepared.

#### EXAMPLE 71

##### (Layered Photoconductor No. 16-1)

One part by weight of a bisazo compound represented by the formula (1-8), 19 parts by weight of tetrahydrofuran, and 6 parts by weight of a tetrahydrofuran solution of a polyvinyl butyral resin (Trade Name: XYHL made by Union Carbide Plastic Company) (5 weight percent) were ground in a ball mill.

To the thus ground mixture were added 104 parts by weight of tetrahydrofuran while stirring slowly. The thus prepared dispersion was coated on the aluminum surface side of an aluminum-evaporated polyester film by a doctor blade, with a wet gap of 35  $\mu\text{m}$ , and was then dried at 80° C. for 5 minutes, whereby a charge generation layer with a thickness of 0.9  $\mu\text{m}$  was formed on the aluminum-evaporated polyester film.

Furthermore, 10 parts by weight of hydrazone compound (2-26), 10 parts by weight of a polycarbonate resin (Trade Name: Panlite K-1300 made by Teijin Limited), 0.002 parts by weight of silicone oil (Trade Name: KF-50 made by The Shin-Etsu Chemical Co., Ltd.) and 80 parts by weight of tetrahydrofuran were mixed to form a solution. This solution was coated on the charge generation layer by a doctor blade with a wet gap of 200  $\mu\text{m}$  and was then dried at 80° C. for 2 minutes and then at 100° C. for 5 minutes, so that a charge transport layer with a thickness of 19.1  $\mu\text{m}$  was formed on the charge generation layer, whereby a layered electrophotographic photoconductor No. 16-1 was prepared.

#### EXAMPLE 72

##### (Layered Photoconductor No. 16-2)

Example 71 was repeated except that hydrazone compound (2-26) was replaced with hydrazone compound (2-20), so that a layered electrophotographic photoconductor No. 16-2 with a charge generation layer with a thickness of 0.9  $\mu\text{m}$  and a charge transport layer with a thickness of 17.8  $\mu\text{m}$  was prepared.

#### EXAMPLE 73

##### (Layered Photoconductor No. 16-3)

Example 71 was repeated except that hydrazone compound (2-26) was replaced with hydrazone compound (2-36), so that a layered electrophotographic photoconductor No. 16-3 with a charge generation layer with a thickness of 0.9  $\mu\text{m}$  and a charge transport layer with a thickness of 18.4  $\mu\text{m}$  was prepared.

#### EXAMPLE 74

##### (Layered Photoconductor No. 16-4)

Example 71 was repeated except that hydrazone compound (2-26) was replaced with hydrazone compound (2-23), so that a layered electrophotographic photoconductor No. 16-4 with a charge generation layer with a thickness of 0.9  $\mu\text{m}$  and a charge transport layer with a thickness of 17.0  $\mu\text{m}$  was prepared.

## EXAMPLE 75

(Layered Photoconductor No. 16-5)

Example 71 was repeated except that hydrazone compound (2-26) was replaced with hydrazone compound (2-30), so that a layered electrophotographic photoconductor No. 16-5 with a charge generation layer with a thickness of 0.9  $\mu\text{m}$  and a charge transport layer with a thickness of 16.2  $\mu\text{m}$  was prepared.

## EXAMPLE 76

(Layered Photoconductor No. 16-6)

Example 71 was repeated except that hydrazone compound (2-26) was replaced with hydrazone compound (2-24), so that a layered electrophotographic photoconductor No. 16-6 with a charge generation layer with a thickness of 0.9  $\mu\text{m}$  and a charge transport layer with a thickness of 19.8  $\mu\text{m}$  was prepared.

## EXAMPLE 77

(Layered Photoconductor No. 16-7)

Example 72 was repeated except that the polyvinyl butyral resin was replaced with a polyester resin (Trade Name: Vylon 200 made by Toyobo Co., Ltd.), so that a layered electrophotographic photoconductor No. 16-7 with a charge generation layer with a thickness of 0.9  $\mu\text{m}$  and a charge transport layer with a thickness of 18.4  $\mu\text{m}$  was prepared.

The thus prepared electrophotographic photoconductors were each charged negatively in the dark under application of -6 kV of corona charge for 20 seconds and the surface potential  $V_s$  (Volt) of each photoconductor was measured by a Paper Analyzer (Kawaguchi Works, Model SP-428). Each photoconductor was then allowed to stand in the dark for 20 seconds without applying any charge thereto, and the surface potential  $V_o$  (Volt) of the photoconductor was measured by the Paper Analyzer. Each photoconductor was then illuminated by a tungsten lamp in such a manner that the illuminance on the illuminated surface of the photoconductor was 20 lux, and the exposure  $E_{1/2}$  (lux second) required to reduce the initial surface potential  $V_o$  (Volt) to  $\frac{1}{2}$  was measured. The exposure  $E_{1/10}$  (lux second) required to reduce the initial surface potential  $V_o$  (Volt) to  $1/10$  was also measured. The results are shown in Table 1.

In order to illustrate the advantages of the present invention, the following comparative layered photoconductors were prepared:

## COMPARATIVE EXAMPLE 1

(Comparative Layered Photoconductor No. 1)

In a vacuum chamber with a vacuum degree of  $10^{-5}$  mmHg, an aluminum base plate was placed above  $N,N'$ -dimethylperylene-3,4,9,10-tetracarboxyldiimide, which served as a charge generating material, in an evaporation source. The  $N,N'$ -dimethylperylene-3,4,9,10-tetracarboxyldiimide was heated to 350° C. and evaporation was permitted to continue for 3 minutes to form a charge generation layer on the aluminum base plate.

A solution consisting of 5 parts by weight of 2,5-bis(4-diethylaminophenyl)-1,3,4-oxadiazole, 5 parts by weight of a polyester resin (Trade Name: Polyester Adhesive 49000 manufactured by Du Pont) and 90 parts by weight of tetrahydrofuran was coated on the charge generation layer and was dried at 120° C. for 5 minutes, so that a charge transport layer with a thickness of

about 10  $\mu\text{m}$  was formed on the charge generation layer, whereby a comparative layered photoconductor No. 1 was prepared.

## COMPARATIVE EXAMPLE 2

(Comparative Layered Photoconductor No. 2)

1.08 parts by weight of Chlorodiane Blue (a benzidine type pigment), which served as a charge generating material, was dissolved in 24.46 parts by weight of ethylenediamine. To this solution was added 20.08 parts by weight of n-butylamine with stirring and 54.36 parts by weight of tetrahydrofuran was then added, whereby a charge generation layer coating liquid was prepared. The charge generation layer coating liquid was coated on the aluminum surface side of an aluminum-evaporated film by a doctor blade, and was then dried at 80° C. for 5 minutes, whereby a charge generation layer with a thickness of about 0.5  $\mu\text{m}$  was formed on the aluminum-evaporated polyester film.

20 A solution of 1 part by weight of 1-phenyl-3-(4-diethylaminostyryl)-5-(4-diethylaminophenyl)-pyrazoline, 1 part by weight of polycarbonate resin (Trade Name: Panlite K-1300 made by Teijin Limited) and 8 parts by weight of tetrahydrofuran was coated on the above-described charge generation layer by a doctor blade and then dried at 80° C. for 2 minutes and then at 100° C. for 5 minutes, so that a charge transport layer with a thickness of about 20  $\mu\text{m}$  was formed on the charge generation layer, whereby a comparative layered photoconductor No. 2 was prepared.

## COMPARATIVE EXAMPLE 3

(Comparative Layered Photoconductor No. 3)

Two parts by weight of 2,7-bis[2-hydroxy-3-(2,4-dimethoxy-5-chlorophenylcarbamoyl)-1-naphthylazo]-9-fluorenone, which served as charge generating material, and 98 parts by weight of tetrahydrofuran were ground in a ball mill to form a dispersion. This dispersion was coated on the aluminum surface side of an aluminum-evaporated polyester film by a doctor blade and was then dried at room temperature, whereby a charge generation layer with a thickness of 1  $\mu\text{m}$  was formed on the aluminum-evaporated polyester film.

45 Two parts by weight of 2,5-bis(4-diethylaminophenyl)-1,3,4-oxadiazole, 2 parts by weight of a polycarbonate resin (Trade Name: Panlite L made by Teijin Limited) and 46 parts by weight of tetrahydrofuran were mixed to obtain a charge transport layer coating solution. This solution was coated on the above-described charge generation layer by a doctor blade and was then dried at 120° C. for 10 minutes, so that a charge transport layer with a thickness of 10  $\mu\text{m}$  was formed on the charge generation layer, whereby a comparative layered photoconductor No. 3 was prepared.

## COMPARATIVE EXAMPLE 4

(Comparative Layered Photoconductor No. 4)

60 One part by weight of a polyester resin (Trade Name: Polyester Adhesive 49000 made by Du Pont), 1 part by weight of 2,7-bis[2-hydroxy-3-(4-chlorophenylcarbamoyl)-1-naphthylazo]-9-fluorenone, which was a fluorenone type bisazo pigment, and 26 parts by weight of tetrahydrofuran were ground in a ball mill to obtain a dispersion.

65 This dispersion was coated on the aluminum surface side of an aluminum-evaporated polyester film by a

doctor blade and was then dried at 100° C. for 10 minutes to form a photoconductive layer with a thickness of 7  $\mu\text{m}$  on the aluminum-evaporated polyester film, whereby a comparative layered photoconductor No. 4 was prepared.

The electrostatic characteristics of those comparative photoconductors were measured under the conditions stated in the examples of the electrophotographic photoconductors according to the present invention. The results are shown in Table 2.

TABLE 1

| Photoconductor | V <sub>po</sub><br>(Volt) | E <sub>1/2</sub><br>(lux · sec) | E <sub>1/10</sub><br>(lux · sec) |
|----------------|---------------------------|---------------------------------|----------------------------------|
| No. 1-1        | -779                      | 1.2                             | 2.6                              |
| No. 1-2        | -915                      | 1.1                             | 2.4                              |
| No. 1-3        | -810                      | 1.2                             | 2.4                              |
| No. 1-4        | -583                      | 0.9                             | 1.8                              |
| No. 2-1        | -734                      | 1.5                             | 3.3                              |
| No. 2-2        | -863                      | 1.3                             | 2.9                              |
| No. 2-3        | -784                      | 1.5                             | 3.1                              |
| No. 3-1        | -751                      | 1.2                             | 2.5                              |
| No. 3-2        | -842                      | 1.1                             | 2.4                              |
| No. 4-1        | -812                      | 1.6                             | 3.6                              |
| No. 4-2        | -865                      | 1.5                             | 3.3                              |
| No. 4-3        | -820                      | 1.5                             | 3.3                              |
| No. 5-1        | -865                      | 2.1                             | 4.4                              |
| No. 5-2        | -1005                     | 2.0                             | 4.3                              |
| No. 5-3        | -964                      | 2.1                             | 4.3                              |
| No. 6-1        | -705                      | 2.3                             | 4.7                              |
| No. 6-2        | -796                      | 2.1                             | 4.4                              |
| No. 7-1        | -870                      | 1.0                             | 2.1                              |
| No. 7-2        | -973                      | 1.3                             | 2.7                              |
| No. 7-3        | -840                      | 1.2                             | 2.4                              |
| No. 8-1        | -473                      | 1.7                             | 3.4                              |
| No. 8-2        | -587                      | 1.6                             | 3.3                              |
| No. 8-3        | -527                      | 1.7                             | 3.3                              |
| No. 9-1        | -790                      | 1.2                             | 2.3                              |
| No. 9-2        | -938                      | 1.2                             | 2.5                              |
| No. 9-3        | -851                      | 1.1                             | 2.3                              |
| No. 9-4        | -944                      | 1.4                             | 2.8                              |
| No. 9-5        | -619                      | 1.0                             | 2.0                              |
| No. 9-6        | -1048                     | 1.3                             | 2.2                              |
| No. 9-7        | -924                      | 1.1                             | 2.2                              |
| No. 10-1       | -742                      | 1.4                             | 3.0                              |
| No. 10-2       | -887                      | 1.4                             | 3.1                              |
| No. 10-3       | -812                      | 1.3                             | 2.8                              |
| No. 10-4       | -902                      | 1.7                             | 3.3                              |
| No. 10-5       | -594                      | 1.3                             | 2.7                              |
| No. 10-6       | -947                      | 1.5                             | 3.1                              |
| No. 10-7       | -886                      | 1.3                             | 2.6                              |
| No. 11-1       | -740                      | 1.2                             | 2.3                              |
| No. 11-2       | -902                      | 1.3                             | 2.6                              |
| No. 11-3       | -829                      | 1.2                             | 2.4                              |
| No. 11-4       | -909                      | 1.4                             | 2.9                              |
| No. 11-5       | -581                      | 1.2                             | 2.6                              |
| No. 11-6       | -969                      | 1.2                             | 2.5                              |
| No. 12-1       | -812                      | 1.5                             | 3.2                              |
| No. 12-2       | -900                      | 1.6                             | 3.5                              |
| No. 12-3       | -860                      | 1.5                             | 3.2                              |
| No. 12-4       | -905                      | 1.8                             | 3.9                              |
| No. 12-5       | -800                      | 1.4                             | 2.8                              |
| No. 12-6       | -800                      | 1.6                             | 3.6                              |
| No. 12-7       | -800                      | 1.5                             | 3.1                              |
| No. 13-1       | -827                      | 2.3                             | 4.5                              |
| No. 13-2       | -1032                     | 2.3                             | 4.7                              |
| No. 13-3       | -915                      | 2.2                             | 4.4                              |
| No. 13-4       | -1018                     | 2.7                             | 4.9                              |
| No. 13-5       | -735                      | 2.0                             | 3.9                              |
| No. 13-6       | -1112                     | 2.5                             | 4.9                              |
| No. 13-7       | -983                      | 2.1                             | 4.3                              |
| No. 14-1       | -600                      | 1.9                             | 3.9                              |
| No. 14-2       | -731                      | 2.1                             | 4.3                              |
| No. 14-3       | -620                      | 1.8                             | 3.7                              |
| No. 14-4       | -742                      | 2.2                             | 4.6                              |
| No. 14-5       | -504                      | 1.7                             | 3.4                              |
| No. 14-6       | -680                      | 2.3                             | 4.7                              |
| No. 15-1       | -812                      | 2.0                             | 4.4                              |
| No. 15-2       | -893                      | 2.1                             | 4.7                              |
| No. 15-3       | -900                      | 2.0                             | 4.3                              |
| No. 15-4       | -895                      | 2.4                             | 5.1                              |

TABLE 1-continued

| Photoconductor | V <sub>po</sub><br>(Volt) | E <sub>1/2</sub><br>(lux · sec) | E <sub>1/10</sub><br>(lux · sec) |
|----------------|---------------------------|---------------------------------|----------------------------------|
| No. 15-5       | -700                      | 1.9                             | 3.8                              |
| No. 15-6       | -985                      | 2.2                             | 4.9                              |
| No. 15-7       | -905                      | 1.9                             | 4.1                              |
| No. 16-1       | -572                      | 1.5                             | 3.1                              |
| No. 16-2       | -730                      | 1.5                             | 3.2                              |
| No. 16-3       | -638                      | 1.4                             | 2.9                              |
| No. 16-4       | -716                      | 1.8                             | 3.7                              |
| No. 16-5       | -441                      | 1.4                             | 2.9                              |
| No. 16-6       | -873                      | 1.6                             | 3.3                              |
| No. 16-7       | -732                      | 1.4                             | 3.0                              |

TABLE 2

| Comparative<br>Photoconductor | V <sub>po</sub><br>(Volt) | E <sub>1/2</sub><br>(lux · sec) | E <sub>1/10</sub><br>(lux · sec) |
|-------------------------------|---------------------------|---------------------------------|----------------------------------|
| No. 1                         | -960                      | 5.4                             | 27.0                             |
| No. 2                         | -603                      | 1.9                             | 4.1                              |
| No. 3                         | -993                      | 5.1                             | 11.0                             |
| No. 4                         | -114                      | 9.6                             | 39.2                             |

As can be seen from Table 1 and Table 2, the layered electrophotographic photoconductors according to the present invention have a higher photosensitivity and a lower residual surface potential than the comparative photoconductors No. 1 through No. 4.

Furthermore, the photoconductors according to the present invention have an advantage over the comparative layered photoconductor No. 2 in that the toxic organic amine is unnecessary for the production thereof.

The photoconductors according to the present invention were each mounted in a commercially available electrophotographic copying machine Ricopy P-500 (made by Ricoh Company, Ltd.) and copying was repeated 10,000 times. Clear copies were made by all the layered photoconductors according to the present invention. This demonstrated that those photoconductors had also excellent durability in repeated use.

What is claimed is:

1. In a layered electrophotographic photoconductor comprising an electroconductive support material and a photoconductive double layer which consists of a charge generation layer and a charge transport layer, the improvement wherein:
  - a. said charge generation layer comprises a charge generating material selected from the group consisting of bisazo pigments of the formula



60 wherein A represents  $-\text{C}_6\text{H}_4-\text{Cl}(\text{o})$ ,  $-\text{C}_6\text{H}_4-\text{Cl}(\text{m})$ ,  $-\text{C}_6\text{H}_4-\text{Br}(\text{o})$ ,  $-\text{C}_6\text{H}_4-\text{Br}(\text{m})$ ,  $-\text{C}_6\text{H}_4-\text{F}(\text{o})$ ,  $-\text{C}_6\text{H}_4-\text{F}(\text{m})$ ,  $-\text{C}_6\text{H}_4-\text{F}(\text{p})$ , or  $-\text{C}_6\text{H}_4-\text{I}(\text{m})$ ; and

- 65 b. said charge transport layer comprises a charge transporting material selected from the group consisting of the hydrazone compounds of the formula



wherein  $R^1$  represents a substituted or non-sub-

3. A layered electrophotographic photoconductor as claimed in claim 1 wherein said charge generating material is



4. A layered electrophotographic photoconductor as claimed in claim 1, wherein said charge generating material is



stituted naphthyl group, a substituted or non-sub- 35  
stituted anthryl group, a substituted or non-sub-  
stituted styryl group, or

5. A layered electrophotographic photoconductor as claimed in claim 1, wherein said charge generating material is



wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other;  $R^2$  represents an alkyl group, a benzyl group; and  $R^3$  represents a phenyl group or a methoxy- 50 phenyl group.

2. A layered electrophotographic photoconductor as claimed in claim 1 wherein said charge generating material is

6. A layered electrophotographic photoconductor as claimed in claim 1, wherein said charge generating material is





7. A layered electrophotographic photoconductor as claimed in claim 1, wherein said charge generating material is

content of said hydrazone compound in said charge transport layer is in the range of 25 to 75 weight percent.



8. A layered electrophotographic photoconductor as claimed in claim 1, wherein said charge generating material is

11. In a layered electrophotographic photoconductor comprising an electroconductive support material and a photoconductive double layer which consists of a



9. A layered electrophotographic photoconductor as claimed in claim 1, wherein said charge generating material is

charge generation layer and a charge transport layer, the improvement wherein:

a. said charge generation layer comprises a charge



10. A layered electrophotographic photoconductor as claimed in claim 1, wherein the thickness of said charge generation layer is in the range of 0.01  $\mu$ m to 5  $\mu$ m and the content of said bisazo pigment in said charge generation layer is in the range of 10 to 100 weight percent and the thickness of said charge transport layer is in the range of 2  $\mu$ m to 100  $\mu$ m and the

generating material selected from the group consisting of bisazo pigments of the formula



wherein A represents  $-C_6H_4-Cl(o)$ ,  $-C_6-$

$-H_4-Cl(m)$ ,  $-C_6H_4-Br(o)$ ,  $-C_6H_4-Br(m)$ ,

$-C_6H_4-F(o)$ ,  $-C_6H_4-F(m)$ ,  $-C_6H_4-F(p)$ , or

$-C_6H_4-I(m)$ ; and

b. said charge transport layer comprises a charge

transporting material selected from the group con-

sisting of the hydrazone compounds of the formula

5

10

15

20

25

30

35

40

45

50

55

60

65



wherein B represents hydrogen, an alkyl group with one to three carbon atoms, an alkoxy group with one to three carbon atoms, a dialkylamino group, halogen, a nitro group, or a hydroxy group, and n represents an integer of 1 to 5, and when n is 2 or more, B can be different or identical to each other.

12. A layered electrophotographic photoconductor as claimed in claim 11 in which the OCH<sub>3</sub> group is in para position.

13. A layered electrophotographic photoconductor as claimed in claim 11 in which B is said alkyl group, said alkoxy group, halogen, nitro or hydroxy.

14. A layered electrophotographic photoconductor as claimed in claim 1 in which R<sup>1</sup> is naphthyl or substituted naphthyl.

15. A layered electrophotographic photoconductor as claimed in claim 1 in which R<sup>1</sup> is anthryl or substituted anthryl.

16. A layered electrophotographic photoconductor as claimed in claim 1 in which R<sup>1</sup> is styryl or substituted styryl.

\* \* \* \* \*

UNITED STATES PATENT AND TRADEMARK OFFICE  
**CERTIFICATE OF CORRECTION**

PATENT NO. : 4 481 271

Page 1 of 2

DATED : November 6, 1984

INVENTOR(S) : Mitsuru HASHIMOTO et al

It is certified that error appears in the above-identified patent and that said Letters Patent is hereby corrected as shown below:

Column 38, line 47; delete "a" (first occurrence only).

line 48; change "alyer" to ---layer---.

Column 39, line 1; change "R<sup>1</sup>-CH=N-N-R<sup>3</sup>" to  
|  
R<sup>2</sup>

$$\text{---R}^1\text{---CH=N---N---R}^3\text{---.}$$

$\text{R}^2$

line 6; after "anthryl group," insert ---or---.

line 7; after "styryl group" change the comma to a semi-colon (;).

lines 8 (which contains a formula) through 14; delete in their entirety.

line 15; delete "other".

after "alkyl group" change the comma to ---or---.

line 16; after "phenyl group" insert a period.

delete "or a methoxy-".

line 17; delete in its entirety.

line 19; after "claim 1" insert ---or claim 11---.

UNITED STATES PATENT AND TRADEMARK OFFICE  
CERTIFICATE OF CORRECTION

PATENT NO. : 4 481 271

Page 2 of 2

DATED : November 6, 1984

INVENTOR(S) : Mitsuru HASHIMOTO et al

It is certified that error appears in the above-identified patent and that said Letters Patent is hereby corrected as shown below:

Column 40, line 2; after "claim 1" insert ---or claim 11---.

line 6; after "claim 1" insert ---or claim 11---.

line 35; after "claim 1" insert ---or claim 11---.

line 46; after "claim 1" insert ---or claim 11---.

Column 41, line 15; after "claim 1" insert ---or claim 11---.

line 34; after "claim 1" insert ---or claim 11---.

line 49; after "claim 1" insert ---or claim 11---.

line 63; after "claim 1" insert ---or claim 11---.

Signed and Sealed this

*Sixth Day of August 1985*

[SEAL]

*Attest:*

DONALD J. QUIGG

*Attesting Officer*

*Acting Commissioner of Patents and Trademarks*